

K. WARGA,  
DECORATING GLASS SURFACES.

APPLICATION FILED AUG. 16, 1916. RENEWED MAY 11, 1918.

1,283,606.

Patented Nov. 5, 1918

Fig. 1



Fig. 2



Witness:

Kenneth Stone.

Inventor:  
Kalman Warga  
By William M. Stone.  
his Attorney.

# UNITED STATES PATENT OFFICE.

KALMAN WARGA, OF BROOKLYN, NEW YORK, ASSIGNOR TO AMERICAN LITHOGRAPHIC COMPANY, OF NEW YORK, N. Y., A CORPORATION OF NEW YORK.

## DECORATING GLASS SURFACES.

1,283,606.

Specification of Letters Patent.

Patented Nov. 5, 1918.

Application filed August 16, 1916, Serial No. 115,195. Renewed May 11, 1918. Serial No. 234,019.

To all whom it may concern:

Be it known that I, KALMAN WARGA, a citizen of the United States, and a resident of the borough of Brooklyn, city of New York, in the county of Kings and State of New York, have invented a certain new and useful Improved Process for Decorating Glass Surfaces, of which the following is a specification.

10 This invention relates to a process for decorating glass surfaces and has for its object to furnish a process of the class specified wherein a plurality of colors or a plurality of characters of design, or both, may be applied to and incorporated with the bodies of glass objects by fusing them thereon in a single fusing operation, without distorting, blistering or clouding either the glass object or the design.

20 With these objects in view I proceed as follows in carrying out my improved process.

Heretofore, in applying by fusing, designs; lettering or the like to glass objects it usually has been considered necessary to fuse each color separately and so build up the multicolor design on the glass by successive firings, an obviously laborious and expensive process. I am aware, however, 30 that it has been proposed to apply a plurality of colors at one time and fix in one firing but by any process known to me this has been an exceedingly precarious process and productive of too high a percentage of 35 failures to permit the process to become of commercial value.

In processes of this general class, while it is possible to apply the color films directly to the object to be decorated, it is preferable 40 and customary to prepare the design upon decalcomania paper, transfer the design in the usual way therefrom to the surface of the glass and then fix by firing.

I preferably follow this general practice 45 in my improved process, employing mineral colors of known constituents but mixing them with the flux in proportions peculiar to my process and with a definite object presently to be pointed out.

50 The design may be conveniently applied to the decalcomania paper by some well known printing process, preferably by lithography. A size of suitable quality may be procured by mixing spirits of turpentine 108 55 parts; balsam of fir 50 parts; sugar of lead

3 parts, and soft flux 1 part, the proportions being approximate. Proper mixing of these ingredients may be attained by heating them together in a water-jacketed container, the water being brought to the boiling point and 60 so maintained until the mixture attains a syrupy consistency when it is cooled and ready for use.

All of the ingredients of the size, of which I have described the method of preparation, 65 which would interfere in any way with the incorporation of the coloring matter with the body of the glass object are of such low carbonizing points as to be driven off or consumed before actual fusion of the color begins, while they may freely escape from their connection with the color. This obviates the formation of gases in the color after it begins fusing and prevents all blistering and clouding of the color. Also the fact that said size is nonsoluble in water enables me to utilize the ordinary decalcomania process and to wash off with water any gum remaining on the design after stripping the decalcomania paper therefrom. 80

The soft flux employed is of known character in the art and may be prepared for use by being moistened with water, heated to about 300 degrees centigrade and then ground to a fine powder. 85

In the drawing accompanying this specification Figure 1 is a cross sectional view of a sheet of decalcomania paper bearing a design prepared in accordance with my improved process. Fig. 2 is a similar sectional 90 view showing the design applied to the glass object. In both views the thicknesses of the several films of color and of the paper and glass are greatly exaggerated.

For purposes of illustration let it be assumed that we wish to produce a three color design on the glass object. The design for the first color is laid upon the stone in the size above described and printed upon the gummed face 5 of the decalcomania paper 4; 100 when the paper is taken from the press the desired first color, 1, in powdered form is dusted upon the face of the paper and so much of the powdered color as covers the sized parts adheres thereto while the rest 105 may be readily removed by a soft brush. The process of printing in size for the second color is then performed over this first color on the paper and that second color, 2, is then dusted upon the face of the paper and the 110

surplus portion removed by a soft brush as already described in connection with the first color. The third printing in size is then performed and the third color, 3, dusted on and 5 the surplus removed. It will be understood that the decalcomania paper is suitably dried after each printing before the succeeding coat of size is applied.

The powdered flux, a small portion of 10 which is used in the size, is also mixed with the glass colors in which the design is to be produced and in said mixing lies the essential features of the present improvement, as the greater the quantity of flux employed 15 relative to the quantity of color, the lower the degree of temperature required for fusing. By taking advantage of this property I am able to fix by fusion the successive colors successively on the glass whereby the 20 colors are prevented from running into one another to the injury or destruction of the design.

That color film 3, which, after the three color design is transferred to the glass, lies 25 next to the glass contains the highest percentage of flux so that when the glass object is heated to fix the design, that color nearest the glass will first fuse and fix itself upon the glass. Then the next color, 2, will be 30 mixed with a lower percentage of flux so that it will fuse after the first color, 3, has fused and fixed itself to the glass and the third or last color, 1, will be mixed with a still lower percentage of flux or none at all 35 so that it will fuse last, after the first and second colors have successively fused and successively fixed themselves to the glass. It will also be obvious, that for transference from the decalcomania paper 4, that color 40 which is to appear uppermost in the design on the glass will be the first one printed on the paper and will have the lowest percentage of flux, also that the color which is to be the bottom color of the design on the glass 45 will be the last one printed on the decalcomania paper and will be mixed with the highest percentage of flux.

Preferably that color which is first printed on the paper will be prepared to have a 50 fusing point about 100 degrees centigrade less than that of the particular glass to which the design is to be applied, and the next color will be prepared to have a fusing point somewhat lower than the fusing point 55 of the first color, say about 50 degrees less by preference. Then the third color to be printed on the paper, over the other two colors, will be prepared with a fusing point about 50 degrees lower than the fusing point 60 of the middle color. If more than three colors are used the difference in fusing temperatures may be less than 50 degrees so as not to have an excessive difference between the lowest and highest.

65 That part of the surface of the glass ob-

ject to which the design or lettering is to be applied is then preferably coated with a fixing agent 6 preferably the size previously described, but for this use, the size is preferably heated only sufficiently to dissolve 70 the sugar of lead.

The decalcomania paper 4, bearing the three color design is then applied to the sized surface of the glass object 7, and the design transferred thereto in the usual manner and the paper removed therefrom. Any portion of the gum 5, from the decalcomania paper may be washed off with water from the design on the glass 7, and the glass object allowed to dry. It is then placed in a 80 leer at a low initial temperature and gradually advanced through the leer to a maximum degree of heat requisite only to produce fusion of that color having the highest fusing point. 85

In passing through the leer the fusing point of that color lying next to the glass is first reached, whereupon that color melts and fixes itself to the glass without disturbing the other two colors. The first color 90 being therefore firmly attached to the glass by fusion, the increasing heat of the leer melts the second color which thereupon fixes itself onto the first color, already fixed on the glass. The further heat of the leer then 95 fuses the third color, without approaching nearer than about 100 degrees to the fusing point of the glass and which color thereupon fixes itself to that middle color just below it. The glass object is then advanced 100 through lower and lower temperatures to nearly atmospheric temperature. Upon withdrawal from the leer the design will be found to be irremovably fixed upon the glass object without any running or mixing 105 of the colors or any distortion of the glass object, or without any blistering or clouding of the design.

In fixing designs or lettering upon bottles or other containers, and sometimes in other 110 cases, it is often desirable to provide a ground for the more distinct relief of a design or lettering and in the same color. In this case I mix the ground color with a proper amount of flux to give that color a 115 melting point some 50 degrees less than that of the superposed design or lettering in the same color upon it. Also I may add a third printing of the same color but with a still higher melting point so as to build up a 120 raised design all in one color.

I claim:

1. The process of fixing designs and the like upon glass objects comprising forming said designs in mineral colors fusible respectively at predetermined successive degrees of heat the highest of which is substantially lower than that necessary to initiate the fusion of the glass object and then fixing said designs by firing. 130

2. The process of fixing designs and the like upon glass objects, consisting in applying to the surface of the glass two or more superposed color films of mineral coloring matter, the material of said films respectively having been previously so compounded as to fuse at temperatures successively increasing from the film nearest the glass to that film most remote from the glass, said film most remote from the glass having a melting point lower than the initial fusing point of the glass and then fixing said color films by firing.

3. The process of fixing designs and the like upon glass objects comprising forming said designs into mineral colors fusible respectively at predetermined successive degrees of heat, the highest of which is substantially lower than that necessary to initiate the fusion of the glass object; then applying to the glass object a fixing agent, nonsoluble in water, the combustible ingredients of which are eliminable by heat of a degree substantially lower than the degree of heat requisite to initiate fusing of the mineral color; then applying the colors upon the fixing agent on the glass object, and finally exposing the glass object to a low degree of heat and gradually increasing such heat to a degree sufficient to produce fusion of the colors and then gradually reducing the heat to a degree approximating atmospheric temperature.

4. The process of fixing designs and the like, upon glass objects, comprising mixing glass colors with a soft flux to make the color matter fusible respectively at successive predetermined degrees of heat substantially lower than the degree of heat requisite to initiate fusing of the glass object to be treated; printing the design, lettering, or the like, upon decalcomania paper in a fixing agent made of spirits of turpentine approximating 108 parts, balsam of fir approximating 50 parts, sugar of lead approximating 3 parts, and soft flux approximating 1 part, heated until reduced to a syrupy consistency; applying the colors to such fixing agent printed on the decalcomania paper; coating the glass object with a fixing agent of the same ingredients, but heated only sufficiently to dissolve the sugar of lead therein; transferring the colors of the design from the decalcomania paper to the coated portion of the glass object, and

subjecting the glass object to a low heat, and gradually increasing such heat to a degree sufficient to produce fusing of the colors, and then gradually reducing such heat to a degree of heat approximating the atmospheric temperature.

5. The process of fixing designs and the like upon glass objects, consisting in applying to the surface of the glass two or more superposed color films of mineral coloring matter, the material of said films, respectively, having been previously so compounded as to fuse at temperatures successively increasing from the film nearest the glass to that film most remote from the glass, said film most remote from the glass having a melting point lower than the initial fusing point of the glass, then slowly heating the glass object to a temperature sufficient to fuse that film of coloring matter having the highest melting point, and then gradually cooling the glass object to near atmospheric temperature.

6. The process of fixing designs and the like upon glass objects, comprised in applying to the surface of the glass two or more color films of mineral coloring matter, the material of said films having been previously so compounded as to fuse respectively at varying temperatures the melting point of that film having the highest fusing point being most remote from the glass and then fixing said color films by firing.

7. Those steps in the process of fixing designs and the like upon glass objects comprising forming said designs in more than one mineral color fusible respectively at predetermined different degrees of heat, the highest of which is substantially lower than that necessary to initiate the fusion of the glass object.

8. Those steps in the process of fixing designs and the like upon glass objects comprising forming said designs in more than one color fusible respectively at predetermined different degrees of heat substantially lower than that necessary to initiate the fusion of the glass object.

Signed at New York, N. Y., this 12th day of August, 1916, before two subscribing witnesses.

KALMAN WARGA.

Witnesses:

STANLEY W. COOK,  
CORNELIUS MUSE, Jr.